

## UNITED STATES PATENT OFFICE

2,658,036

## COMPOSITION FOR PREVENTING DEPOSITION AND CORROSION IN OIL WELL EQUIPMENT

Clark D. Core, Seguin, and Edward N. Jones, Pettus, Tex.; said Core assignor to Texas Acidizers, Incorporated, Seguin, Tex., a corporation of Texas

No. Drawing. Application July 19, 1950,  
Serial No. 174,788

5 Claims. (Cl. 252—8.55.)

1

This invention relates to compositions for use in increasing the efficiency and productivity of oil, gas or water producing wells.

The primary object of this invention is to provide compositions which are more effective in simultaneously preventing corrosion and scale deposition on the metal surface of well equipment, such as casing, tubing, surface connections, flow lines, separators, heaters and tanks than the conventional products presently employed.

Most fluids that come out of earth formations contain many complex inorganic as well as organic chemicals which include compounds of calcium, magnesium, potassium, sodium, iron, carbon, hydrogen, barium and sulphur. While the compounds are trapped in the earth formation, they exist in the fluids in a state of equilibrium which can be disturbed by changes of heat and pressure. When the well is produced, the fluids leave the relatively high temperature and pressure conditions found at the formation and ascend toward the surface of the earth while the temperature and pressure decrease. The equilibrium so upset causes the formation of new compounds, such as carbonic acid and acetic acid, which have a marked corrosive effect on steel, and also causes the formation of compounds which precipitate out upon the steel as a hard scale deposit. Calcium carbonate, calcium sulphate, magnesium sulphate and iron sulphide are several of the compounds which precipitate out as scale. The deposition of the scale compounds and the corrosive compounds remains on the metallic equipment until holes form therein, making immediate replacement necessary. This not only interrupts the production in the well, but also requires costly replacements, particularly in the case of high pressure wells where even one small hole can start a series of costly consequences. Therefore, there is a constant demand in this art for compositions which will simultaneously prevent corrosion and also prevent the depositions of hard scale on the well equipment. The present composition effectively performs this dual function in a manner not heretofore possible with the many compositions presently available on the market.

One of the important ingredients in the present composition is a water-soluble, alkali metal arsenite, such as sodium or potassium arsenite.

As stated hereinabove, it is not only necessary to provide a corrosion inhibitor which will effectively cover the metallic well equipment, but also an ingredient which will remove existing scale

2

and prevent further scale deposition inasmuch as the destruction of well equipment is due to a combination of both the corrosion of the equipment by the acids in the well fluids and the scale deposition on the equipment. Accordingly, the present composition includes a water-soluble, alkali metal hexametaphosphate, such as sodium or potassium hexametaphosphate, which accomplishes this purpose by holding in solution in proper chemical equilibrium the compounds that would otherwise precipitate to form the scale. The sodium hexametaphosphate forms soluble complex compounds with the scale-forming compounds already in solution, the complex compounds being carried harmlessly out of the well equipment in solution with the fluids being produced.

It is well known in this art that crude oil or paraffin films form upon the surfaces of the metal equipment which act as insulation between the metal surface and the treating solutions, and that this is further aggravated by the presence of resistant emulsions of the water-oil and oil-water type. Accordingly, an effective composition for preventing deposition of scale and corrosion must also include an ingredient which will effectively remove the crude oil or paraffin film from the metal surfaces and at the same time effectively break up the resistant emulsions. Experimentation has been conducted with a number of detergents or wetting agents for incorporation with the arsenite and hexametaphosphate, but it has been found that only a few of these wetting agents are really effective for the dual purpose of removing the crude oil or paraffin film and the breaking up of the resistant water-oil and oil-water emulsions. Certain of the well-known Aerosol compounds have been employed to advantage. Aerosol OS has been found to have the best properties, while it has also been found that Aerosol MA, Aerosol AY and Aerosol IB could also be employed in the composition. Aerosol OS is a water soluble wetting agent or detergent otherwise known as isopropyl naphthalene sodium sulfonate, Aerosol MA is dihexyl sodium sulfosuccinate, Aerosol AY is diamyl sodium sulfosuccinate, and Aerosol IB is diisobutyl sodium sulfosuccinate.

It will thus be seen that the basic composition herein provided for preventing deposition of scale and corrosion in oil well equipment comprises a mixture of an alkali metal arsenite, an alkali metal hexametaphosphate, and a wetting agent effective for the removal of crude oil or paraffin film and for the breaking up of oil-water and

water-oil emulsions. This composition may be a dry or solid composition or may be an aqueous solution depending upon the manner of application. The examples which follow illustrate the proportions of the ingredients employed:

## EXAMPLE I

|                                       | Per cent by weight |
|---------------------------------------|--------------------|
| Sodium arsenite, 40% aqueous solution | 4.0-45.0           |
| by weight                             | 10                 |
| Sodium hexametaphosphate              | 4.0-45.0           |
| Aerosol OS                            | 0.4                |
| Remainder—Water.                      |                    |

As the corrosion and scale deposition problems vary greatly in different areas, chemical analysis of the well fluids should be made to determine the variations which must be made in the proportions of the above ingredients. In the case of highly corrosive wells in which very little scale develops, it would be necessary to increase the arsenite concentration and decrease the phosphate concentration correspondingly. On the other hand, if a well has extreme scale development and very little corrosion, the phosphate concentration should be increased and the arsenite concentration correspondingly decreased.

Inasmuch as aldehydes, such as formaldehyde, act as corrosion inhibitors in metallic oil well equipment, and particularly because of a reaction between formaldehyde and hydrogen sulphide in the well fluid to produce a protective film, formaldehyde may be added to the above composition to replace some of the water and the preferred percentage by weight of the added formaldehyde is 2.0%.

The preferred composition and one which has proven highly effective in widespread areas is given in the following example:

## EXAMPLE II

|                                                       | Per cent by weight |
|-------------------------------------------------------|--------------------|
| Sodium arsenite, 40% by weight of an aqueous solution | 45.0               |
| Sodium hexametaphosphate                              | 4.0                |
| Aerosol OS                                            | 0.4                |
| Remainder—Water.                                      |                    |

It will be understood that the above compositions can be administered a number of different ways, but preferably will be injected into the annular space between the well tubing and the long string of casing. The composition trickles down the metallic surfaces of the well equipment to the bottom of the tubing and is picked up in small quantities, but continuously, by the well fluids ascending inside of the tubing.

Instead of the aqueous solutions mentioned hereinabove, a solid mixture of the ingredients, either in stick or pellet form, may be administered in the oil well, and the following example gives the ingredients in their proper percentage by weight for the solid composition:

## EXAMPLE III

|                                 | Per cent |
|---------------------------------|----------|
| Sodium arsenite powder          | 24-71    |
| Sodium hexametaphosphate powder | 24-71    |
| Aerosol OS powder               | 2        |
| Starch                          | 3        |

The starch is used as a binder and a small amount of water is used initially to dissolve the

starch and mold the mixture, after which the water is expelled by heat evaporation.

Thus, it will be seen that novel compositions are provided which, due to their power to remove as well as prevent the formation of scale depositions in well tubing, surface connections and flow lines, free and unobstructed flow of the well fluids is obtained throughout substantially the entire productive life of the well. Inasmuch as these compositions also contain surface-active materials which not only remove crude oil and paraffin deposits on the metallic equipment, but also act as demulsification agents for effectively breaking up the oil-water and water-oil emulsions normally found in wells, both the corrosion inhibiting arsenites and the scale preventing hexametaphosphates can at all times perform their desired functions effectively.

While preferred embodiments of the present composition have been described hereinabove, it will be understood that minor variations in the composition can be made by those skilled in the art without departing from the spirit of the invention or the scope of the appended claims.

Having described the invention, what is claimed as new is:

1. A composition for removing and preventing scale deposition and preventing corrosion in oil well equipment comprising 4-45% by weight of a 40% aqueous solution of an alkali metal arsenite, 4-45% by weight of an alkali metal hexametaphosphate and a minor amount of surface-active demulsification agent, the balance being water.

2. The composition of claim 1 wherein said demulsification agent is selected from the class consisting of isopropyl naphthalene sodium sulfonate, dihexyl sodium sulfosuccinate, diamyl sodium sulfosuccinate and diisobutyl sodium sulfosuccinate.

3. The composition of claim 1 wherein said arsenite is sodium arsenite and said hexametaphosphate is sodium hexametaphosphate.

4. A composition for removing and preventing scale deposition and preventing corrosion in oil well equipment comprising 4-45% by weight of a 40% aqueous solution of sodium arsenite, 4-45% by weight of sodium hexametaphosphate, and a sufficient amount of isopropyl naphthalene sodium sulfonate to act as a demulsification agent.

5. The composition of claim 4 wherein the ingredients are present in the following percentages by weight: sodium arsenite, 40% by weight aqueous solution, 4.0-45.0%; sodium hexametaphosphate 4.0-45.0%, isopropyl naphthalene sodium sulfonate 0.4%, remainder water.

CLARK D. CORE.  
EDWARD N. JONES.

## References Cited in the file of this patent

## UNITED STATES PATENTS

| Number    | Name         | Date           |
|-----------|--------------|----------------|
| 935,695   | Schultze     | Oct. 5, 1909   |
| 1,877,504 | Grebe et al. | Sept. 13, 1932 |
| 1,903,041 | Hall et al.  | Mar. 28, 1933  |
| 2,204,580 | De Groote    | June 18, 1940  |
| 2,262,737 | De Groote    | Nov. 11, 1941  |
| 2,426,318 | Menaul       | Aug. 26, 1947  |
| 2,429,594 | Case         | Oct. 28, 1947  |
| 2,468,163 | Blair et al. | Apr. 26, 1949  |